

June 14, 1960

L. PÉRAS  
MANUFACTURE OF LOW-TENSION SPARKING PLUGS  
FOR INTERNAL COMBUSTION ENGINES  
Filed Jan. 2, 1957

2,940,221

*Fig. 1*



*Fig. 2*



# United States Patent Office

2,940,221  
Patented June 14, 1960

1

2,940,221

## MANUFACTURE OF LOW-TENSION SPARKING PLUGS FOR INTERNAL COMBUSTION ENGINES

Lucien Péras, Billancourt, France, assignor to Régie Nationale des Usines Renault, Billancourt, France

Filed Jan. 2, 1957, Ser. No. 632,048

Claims priority, application France Jan. 11, 1956

2 Claims. (Cl. 49—81)

Many forms of low-tension sparking plug electrodes have already been proposed, wherein the spark occurs across two electrodes by the discharge of a condenser to ignite the air-fuel mixture of internal combustion engines. The problem of incorporating an insulator between the electrodes, due to the very narrow gap available (i.e. from 0.004" to 0.012") is extremely difficult to solve and reduces the range of materials that can be used for this purpose inasmuch as this insulator must have the property of enabling the spark to "glance off" on its surface while offering a convenient mechanical and thermal resistance thereto.

Now this invention relates more particularly to an improved method of manufacturing the insulated electrode unit of low-tension sparking plugs, wherein the insulator consists of glass, notably borosilicated glass.

According to the present invention, the glass is ground to a fine powder and forms a suspension in water or in another organic liquid, this suspension having a pasty consistency. Then, this paste is either applied with a brush or gun-sprayed on to the surface of the metal parts, the latter being accurately scoured and slightly oxidized beforehand by rapidly heating them to dark red heat. After the suspension liquid has evaporated off, the coated parts are heated in atmospheric air or in a nitrogen atmosphere at such temperature that the glass particles melt and form a continuous vitrified or glazed film adhering strongly on the metal surfaces. By applying several coats of glass alternating with heating steps it is possible to form relatively thick glass layers on the metal. These electrodes are assembled upon completion of the vitrification, when the hot mass of glass has a pasty consistency, whereby it may flow back, both in and outside, to fill the space between the electrodes.

The application of this method to a conventional electrode arrangement is illustrated by way of example in the accompanying drawing, wherein Fig. 1 shows a pair of concentric electrodes 1, 2 coated separately as set forth hereinabove, then dried, glazed and disposed in the proper relative positions when the mass of hot, pasty glass flows back in the space 3 between the electrodes so as to fill it. When the assembly has cooled down to room temperature the lower face is ground slightly to remove any excess material which may have flowed outwards and to form a spark gap level with the concentric electrodes.

This method of applying a glass insulation on low-tension sparking plug electrodes may be associated with the combined use of another insulating material. In this case, the glazed or vitrified electrodes are ground and lapped.

Figure 2 of the drawing illustrates in axial section an electrode assembly constituting a typical example of the simultaneous use of the two insulators.

This assembly comprises two electrodes, i.e. a hollow

2

cylindrical electrode 4 and a disc-shaped electrode 7. The former has its inner surface bevelled outwards at its lower end. In this electrode 4, the insulating material 5 is cast in a heated pasty condition and consists, as already explained, of a powder glass suspension in water or other organic liquid. Then, the assembly is heated to melt the glass. Upon completion of the cooling step, the lower face of the electrode is lightly ground until a surface is obtained wherein the metal electrode 4 appears in the form of a thin annulus about 0.016" thick around a wider annulus of insulating material. Then, a mica washer 6 is so applied on this surface that the latter is engaged by the upper face of the washer up to the bevelled portion. Then the other electrode 7 is placed against the washer 6 and held in position by a central rod 8 of conducting material and a nut 9.

I claim:

1. The method of manufacturing a surface discharge spark plug for operation with a discharge condenser in low tension ignition installations which consists of providing a first metallic electrode having an axial bore and a sparking surface and a second metallic electrode having a sparking surface to be assembled coaxially with the first electrode with their sparking surfaces closely spaced and substantially flush and providing insulating material comprising borosilicated glass to be used as an insulating core between the electrodes, and to form a surface substantially coplanar with the sparking surfaces prior to assembly of the electrodes, reducing the glass to a powdered state, adding liquid to the powdered glass to form a composition of a substantially viscous consistency, applying the composition to the electrode surfaces to be assembled, prior to assembly thereof, treating the electrodes in an unassembled condition with heat sufficient to melt the glass particles and fuse them thereby to vitrify the composition, repeating the application of the composition and the vitrification thereof to form successive thin layers of insulating material on the electrodes, heating the electrodes in an unassembled condition with all of the layers of insulating material thereon sufficiently to cause the insulating material to assume a plastic state in preparation for assembling the electrodes, assembling the electrodes by disposing them coaxially and moving them in a direction opposite to each other after a final application and vitrification of the composition while the composition is in a heated and plastic state, and cooling the assembled electrodes.

2. The method according to claim 1, in which prior to the application of the composition to the electrode surfaces the electrodes are oxidized by rapidly heating them to a dark red.

## References Cited in the file of this patent

### UNITED STATES PATENTS

|    |           |              |               |
|----|-----------|--------------|---------------|
| 55 | 1,562,533 | Weintraub    | Nov. 24, 1925 |
|    | 1,775,218 | Thurneyssen  | Sept. 9, 1930 |
|    | 2,125,315 | Ronci        | Aug. 2, 1938  |
|    | 2,136,052 | Hurley       | Nov. 8, 1938  |
| 60 | 2,248,644 | Reger et al. | July 8, 1941  |
|    | 2,293,381 | Carington    | Aug. 18, 1942 |
|    | 2,399,770 | Taylor       | May 7, 1946   |
|    | 2,422,628 | McCarthy     | June 17, 1947 |
|    | 2,429,955 | Goldsmith    | Oct. 28, 1947 |
| 65 | 2,436,644 | Halstead     | Feb. 24, 1948 |
|    | 2,549,504 | Messana      | Apr. 17, 1951 |
|    | 2,560,593 | Pask et al.  | July 17, 1951 |
|    | 2,657,248 | Smits        | Oct. 27, 1953 |
|    | 2,709,147 | Ziegler      | May 24, 1955  |